

J. C. DAVIS.

## ART OF MAKING MOLDS.

APPLICATION FILED DEC. 16, 1912.

1,167,889.

Patented Jan. 11, 1916.



**WITNESSES:**

WITNESSES.  
J. M. Baker.  
Anna Westman.

**INVENTOR**

INVENTOR  
James Carey Davis  
BY  
Paul Carpenter  
ATTORNEY

# UNITED STATES PATENT OFFICE.

JAMES CAREY DAVIS, OF HINSDALE, ILLINOIS, ASSIGNOR TO AMERICAN STEEL  
FOUNDRIES, OF CHICAGO, ILLINOIS, A CORPORATION OF NEW JERSEY.

## ART OF MAKING MOLDS.

1,167,889.

Specification of Letters Patent. Patented Jan. 11, 1916.

Application filed December 16, 1912. Serial No. 736,935.

To all whom it may concern:

Be it known that I, JAMES CAREY DAVIS, a citizen of the United States, and a resident of Hinsdale, in the county of DuPage and 5 State of Illinois, have invented certain new and useful Improvements in the Art of Making Molds, of which the following is a specification.

My present invention relates in general to 10 the art of making castings and more particularly to the production of castings involving one or more of the following features: the use of hard or temperable metal; the use in different parts of the casting of 15 different metals or of different qualities of the same metal; the distribution of parts of varying thicknesses; or a casting which from its prospective use must not be distorted nor vary from its predetermined form; an example of a casting for the production of 20 which my present improvements are particularly available being cast steel car wheels having a tempered thread portion formed of hard manganese steel, an enlarged center 25 formed of relatively soft steel, and a relatively thin web.

In my foundry practice one of the main difficulties which I have found it necessary 30 to overcome in the making of cast steel wheels, such as are produced by the process disclosed in Letters Patent of the United States No. 727103 issued to me, is the relatively high foundry loss, both of molds and 35 of wheels, owing to cracks or fracture, the latter often accompanied by a displacement 40 of a portion of the mold or other distortion, due to difficulty in obtaining a binder for the sand which will be effective under varying operating conditions, and more particularly a binder which may be employed 45 in such a way as to allow the rapid production of molds which is prerequisite to the production of cast steel wheels on a commercial basis under modern foundry conditions.

The principal objects of the present invention are the provision of an improved mold, and a method of and an apparatus for making the same which will so hasten the drying 50 of the mold that a minimum length of

time must necessarily elapse between the making of the mold and the use thereof; the production of a green sand mold having a hard, dry, and tough skin on the surface without affecting interior and thence the 55 desired porosity of the mold whereby ventilation of the mold may be maintained during the act of pouring without in turn affecting such hard dry surface, and the production of green sand molds having a dex- 60 trin or equivalent mixture which may be rapidly dried and used practically immediately after making, together with such further objects as may hereinafter appear.

In carrying out the manufacture of cast 65 steel wheels, and in connection therewith the making of molds for casting such wheels, I have found that green sand when properly mixed with dextrin may be used to form a mold that will dry out upon exposure to 70 atmospheric air and harden in due course, provided a too great degree of humidity is not present in the atmosphere, the time requisite for drying being somewhat dis- 75 proportionate to the humidity of the atmosphere. Such air drying, however, tends to harden the mold throughout and does not give the skin drying effect, which is one of the objects which I most seek to attain, since such skin drying does not affect the 80 porosity of the inner part of the mold. I have found after exhaustive experiments that when a blast of air is directed toward the face of the mold the desired skin drying effect is produced and the desired super- 85 ficial hardness is attained in a very short time, without affecting the inner porosity of the mold, provided that the following conditions be carefully observed, first, that the air is supplied at the proper tempera- 90 ture, under the proper pressure, for the proper length of time and in such a manner that it is properly distributed.

In the accompanying drawing I have 95 illustrated, somewhat diagrammatically, a preferred form of apparatus employed by me for artificially drying the molds, wherein—

Figures 1 and 2 are respectively an eleva- 100 tional and a plan view of the apparatus;

Fig. 3 is a view of a detail of construction; and Fig. 4 is a vertical section through the mold shown at the right hand side of Fig. 1.

Referring first to Fig. 1 of the drawing, it will be observed that I have here indicated a flask, 10, containing a mold member, which may be supported in any convenient manner as by rails, 11, from the floor. For the purpose of subjecting the mold member, to a diffused current of heated air under pressure I employ a hood or cover, 12, the bottom of which is preferably raised by legs, 13, a slight distance above the top of the flask, in order to permit free exit of the air. The top, 12<sup>a</sup> of the cover, 12, has an opening to receive a supply pipe, 14, which is preferably provided with a slip joint, 14<sup>a</sup>, to facilitate the adjustment of the pipe with relation to the opening of the hood. As a means for supplying air under pressure to the supply pipe 14 I employ a blower, 15, which may be driven in any convenient manner as by a belt driving the pulley, 16, (see Fig. 2). As means for preheating the air supplied to the blower I employ a heater 17 connected thereto by a pipe 18. For the purpose of regulating the temperature of the air passing through the pipe 18 to the blower 15 I utilize a cold air inlet 19 (see Fig. 2) controlled by a damper 20. A thermometer may be arranged between the blower 16 and the cover 12, as indicated at 21, to indicate the temperature of the air supplied to the cover.

Referring now more particularly to Figs. 3 and 4, it will be observed that in order to diffuse the blast of air as it enters the hood, 12, I preferably employ a deflector, 22, which may be supported from the top, 12<sup>a</sup>, of the hood in any convenient manner such as by straps, 23. In making molds according to my improved process I find it preferable to supply the air to the hood, 12, at a temperature between 140 degrees and 200 degrees F., substantially, under a pressure of about three ounces, for a period of about ten minutes, and, in the case of molds for making car wheels and the like, to spread the air current by means of a deflector just below the opening in the supply pipe whereby it may be radiated horizontally and strike all parts of the mold substantially equally and with a softened effect as it proceeds toward the lower rim of the hood where it is vented to the atmosphere.

By carrying out the drying process in the manner just described, I find that I am able to form a tough, dry, tenacious skin on the moist mold diagrammatically shown in Fig. 4 by means of the stippled portion 30, which will maintain the form thereof adequately for casting purposes, without substantially affecting the inner porosity of the mold, thus permitting the rapid production and

immediate use of molds, with few if any failures and comparable negligible loss of castings, thus greatly reducing the expenses heretofore incident to the production of cast wheels owing to mold portions becoming fractured and displaced with consequent imperfections in the wheel treads and rims rendering the cast wheels worthless except for scrap metal.

Having thus described my invention and illustrated its use, what I claim as new and desire to secure by Letters Patent is:

1. The method of producing a mold having a metal molding surface composed of a mixture of sand and dextrin, which consists in subjecting the metal molding surface to a current of heated air under pressure.

2. The method of drying molds by means of air, which consists in subjecting the surface of the mold to a current of heated air under pressure of about three ounces.

3. The method of producing a mold having a metal molding surface composed of a mixture of sand and dextrin, which consists in subjecting the metal molding surface to a current of heated air under pressure for a period of about ten minutes.

4. The method of drying molds by means of air, which consists in subjecting the surface of the mold to a current of heated air under pressure at a temperature between substantially 140 degrees and 200 degrees Fahrenheit.

5. The method of producing a mold having a metal molding surface composed of a mixture of sand and dextrin, which consists in subjecting the metal molding surface to a regulated current of heated air under pressure.

6. The method of producing a mold having a metal molding surface composed of a mixture of sand and dextrin, which consists in subjecting the metal molding surface to a distributed current of heated air under pressure.

7. The method of producing a mold having a metal molding surface composed of a mixture of sand and dextrin, which consists in subjecting the metal molding surface to a current of heated air under pressure at a temperature and for a period of time sufficient to form a relatively dry skin on such surface.

8. The method of producing a mold having a metal molding surface composed of a mixture of sand and dextrin, which consists in subjecting the metal molding surface to a current of heated air under pressure at a temperature and for a period of time sufficient to form a relatively dry skin on such surface without drying and thereby affecting the inner porosity of such mold.

9. The method of drying molds by means of air, which consists in subjecting the sur-

face of the mold to a current of air heated to between 140 degrees and 200 degrees Fahrenheit, substantially, such air being supplied under a pressure of about three ounces for a period of about ten minutes.

In testimony whereof I have hereunto

signed my name in the presence of the two  
subscribed witnesses.

JAMES CAREY DAVIS.

Witnesses:

MARTHA WESTMAN,  
PAUL CARPENTER.